

# UNITED STATES PATENT OFFICE.

WILLIAM H. ALLEN, OF DETROIT, MICHIGAN.

## TREATMENT OF IRON AND STEEL TO PREVENT CORROSION.

1,260,740.

Specification of Letters Patent. Patented Mar. 26, 1918.

No Drawing.

Application filed August 2, 1917. Serial No. 184,041.

*To all whom it may concern:*

Be it known that I, WILLIAM H. ALLEN, a citizen of the United States, and residing at Detroit, in the county of Wayne and State of Michigan, have invented a new and Improved Treatment of Iron and Steel to Prevent Corrosion, of which the following is a specification.

This invention relates to the treatment of articles of iron or steel whose surfaces have been treated to change them from metallic iron to phosphates of iron; and its object is a process whereby such portions of the surfaces, which, by reason of improper or ineffective actions of the compounds of phosphorus employed to produce such surfaces are not rendered non-corrodible under the actions of the elements, may be rendered inactive under such conditions.

When articles of iron or steel are treated with soluble acid phosphates according to the directions set forth in the patents to Coslett, No. 870,937, dated November 12, 1907, and to Richards, No. 1,069,903, dated August 12, 1913, for some reason as yet undetermined, they sometimes rust under water or when exposed to moist air. The rusting usually occurs in very small spots or specks and therefore it is possibly due to the formation (segregation) of hydrates of iron, or other compounds capable of causing rusting occluded in the phosphatic surfaces of the metal articles or formed on such surfaces.

In order to render these undesirable compounds of iron inactive, that is, no longer capable of causing rusting, the articles which have been treated with soluble acid phosphates are placed in an approximately

five per cent. aqueous solution of ferrocyanid or ferricyanid, preferably ferrocyanid of sodium or potassium, for a short time, after which they are removed, dried and finished in any desired manner.

By this treatment, the small amounts of iron compounds which may cause rusting and which are occluded in the phosphatic surfaces of the articles being treated, are changed to iron ferro- or ferricyanid, possibly a mixture of the two and therefore non-corrodible.

I claim:

1. The method of preventing the rusting of surfaces of articles of iron and steel which have been changed in part to phosphates of iron, which consists in immersing such articles in an aqueous solution of an iron cyanid of an alkali-metal.

2. The method of preventing the rusting of surfaces of articles of iron and steel which have been changed in part to phosphates of iron, which consists in immersing such articles in a solution of an iron cyanid of potassium.

3. The method of preventing the rusting of surfaces of articles of iron and steel which have been changed in part to phosphates of iron, which consists in immersing such articles in a solution of ferrocyanid of potassium.

4. The method of preventing the rusting of surfaces of articles of iron and steel which have been changed in part to phosphates of iron which consists in immersing such articles in an aqueous solution of a double cyanid of iron and an alkaline earth metal.

WILLIAM H. ALLEN.